

## UNITED STATES PATENT OFFICE

2,146,294

## METHOD OF TREATING MATERIALS CONTAINING SULPHUR

Carle R. Hayward, Quincy, Mass.

No Drawing. Application October 7, 1936,  
Serial No. 104,503

2 Claims. (Cl. 75—77)

This invention relates to a method of treating metallic by-products or waste materials containing sulphur, such as lead battery plates, roasted or sintered lead concentrates, drosses and like materials in which the lead exists in whole or in part as sulphate.

In the usual methods of smelting and recovering lead products, the presence of sulphur causes the formation of matte or dross which requires reworking. This involves additional expense of operations and usually some loss of the lead content. The presence of sulphur also necessitates carrying out such operations at higher temperatures than would be required if all the lead were present as oxide.

It is accordingly an object of this invention to provide a method for the more convenient, economical and effective recovery of lead or of lead products from waste materials containing lead, and particularly from those which contain more or less lead sulphate or sulphate-bearing compounds. It is also an object to provide a method which shall be adaptable to the practices and equipment commonly employed in the art of recovering lead. Other objects will appear from the following disclosure.

In accordance with this invention, it is found that sulphate-bearing materials, in which the sulphate is in substantially water-insoluble form, such as lead sulphate, the sulphur content may nevertheless be removed by converting the sulphate component into a water-soluble form and then dissolving and leaching it from the residual mass of material with which it has been associated. If a part or all of the sulphur is present as sulphide, as in concentrates from sulphide lead ores, it may be first oxidized to the insoluble sulphate, preliminary to the conversion to soluble sulphate. It is found that such conversion of the insoluble sulphate to soluble sulphate, together with dissolution of the soluble sulphate thus formed, leaves the surface of the residual lead or lead-containing material which has been thus reacted upon in an open, porous condition. Therefore, further penetration of the mass by the converting reagent may be readily effected so as to permit its further reaction upon the insoluble sulphate, and the soluble sulphate thus formed may be readily dissolved and removed. In this way the conversion and dissolution of the sulphur-bearing component of the material is progressive throughout the mass or lumps, etc. of material under treatment, is easily effected, and substantially complete conversion of large in-

dustrial quantities may be economically accomplished.

More particularly, it is now found that water solutions of the alkali metal hydroxides, or weak alkaline salts of the alkali metals (such as caustic soda and sodium carbonate) when applied to masses of materials containing insoluble sulphates, such as lead sulphate, are reactive with the sulphate radical to form the corresponding alkali metal sulphate. The latter dissolves in the solution (or water) and leaves a heavy metallic residue or reaction product which is in a porous condition, such that successive portions of the alkaline solution may penetrate into and through the sulphate mass, removing the sulphate and leaving a porous mass of the reaction product of lead, such as the carbonate and/or oxide.

The porous mass as thus formed may be more completely separated from the soluble or dissolved sulphate by washing in water. It is then in a condition substantially free from sulphate and sulphur, and in which it may be readily smelted and reduced to the condition of free metal or developed to such other form as may be desired. For example, the completely desulphated mass may be fused with a reducing agent, with or without the addition of fluxes, to reduce and recover the lead. Other reducible components which may be present in the charge, such as antimony, may also be recovered at the same time, by appropriate treatment in the usual ways.

In this connection, the flux compositions and methods of procedure described in my United States Patent No. 1,804,054 may be advantageously employed. When operating upon scrap battery plates in this manner temperatures of 700 to 800° C. have been satisfactorily employed, high recoveries of lead and antimony have been effected, and but little dross or fume is encountered.

In a typical example of the practical application of my invention, scrap battery plates may be used, which have been "sulphated" so as to contain a considerable deposit or formation of lead sulphate, and a high recovery yield of the lead content has been obtained.

Thus a pile of the scrap battery plates may be leached with the reagent solution or the charge may be immersed in the alkaline solution in a suitable tank. The solution is conveniently made up with normal sodium carbonate or soda ash, either dilute or concentrated but preferably at or

approximating saturation at atmospheric temperature.

The reagent solution may be passed over and through the mass by suitable circulation, as by pumping, or the charge may be left submerged for a sufficient time to permit complete penetration and conversion of the insoluble sulphate to soluble sulphate form by the progressive penetration and conversion of the sulphate components of the mass or charge as a whole. The time required will depend upon the size, composition and physical characteristics of the material under treatment. But it may be determined and controlled, by removing the initial reagent solution, washing until the wash waters are substantially free from soluble sulphate, treating with fresh alkali solution and then testing this for sulphates. When no further tests for sulphates are obtained the charge may be considered as free from its sulphur content.

A suitable, rapid, and in some respects more convenient procedure, is to subject a succession of charges or a continuous stream of the material containing insoluble sulphate to a counter-current of the alkali reagent solution, which may be readily effected in known ways.

The resulting impregnated, converted and leached product thus obtained contains substan-

tially no sulphur as sulphate, but is made up primarily of free metallic lead, lead oxides, salts and boric salts or hydrates of lead which may be readily reduced to the free metal in known ways. It is of an open porous texture, and in a condition suitable for reconversion and reuse in any of the many forms in which lead and lead compounds are commercially desired or required, in highly satisfactory condition.

I claim:

1. A method of treating roasted or sintered sulphide lead ore concentrates, in massive or lump condition, which comprises subjecting the same directly and without mechanical crushing or grinding to an alkaline aqueous solution of an alkali metal compound to form soluble sulphate, removing said soluble sulphate, and smelting the residue thus obtained under reducing conditions.

2. A method of treating materials composed substantially of water-insoluble metal sulphate, in massive or lump condition, which comprises subjecting the same directly and without mechanical crushing or grinding to an alkaline aqueous solution of an alkali metal compound to form soluble sulphate, removing said soluble sulphate, and smelting the residue thus obtained together with a flux under reducing conditions.

CARLE R. HAYWARD.